

## UNITED STATES PATENT OFFICE

WILHELM GAUS, OF LUDWIGSHAFEN-ON-THE-RHINE, GERMANY, ASSIGNOR TO I. G. FARBEININDUSTRIE AKTIENGESELLSCHAFT, OF FRANKFORT-ON-THE-MAIN, GERMANY, A CORPORATION OF GERMANY

## MOTOR FUEL

No Drawing. Application filed May 7, 1926, Serial No. 107,484, and in Germany May 8, 1925.

It is well known that petroleum distillates or products of cracking processes which are marketed as gasoline and the like, are very much inclined to "knocking" when used as motor fuels.

I have now found that this great drawback can be diminished or even completely removed by an addition of methanol to gasoline. Comparatively small quantities of 10 methanol, generally not over 12 per cent by volume, are sufficient for this purpose so that the calorific power of the fuel is not diminished to any substantial degree.

Preferably the methanol is employed in 15 the anhydrous state, as methanol containing water is only slightly soluble in gasoline. In order to further increase the solubility of methanol, mixing facilitators such as for example higher aliphatic alcohols, ketones and 20 the like, may be added. Crude synthetic methanol containing isobutyl alcohol and the like, may be employed as it is obtained in its manufacture in the process according to the present invention.

25 For example, valuable fuel mixtures are obtained by mixing 96 parts, by volume, of American gasoline of 0.75 specific gravity with 4 parts of anhydrous methanol or by mixing 88 parts of gasoline with 12 parts of 30 crude synthetic methanol about two thirds of which consists of methanol and about one third of which consists of products of a higher order than methanol. The composition of crude synthetic methanol after removal of water is for example about as follows:—72 per cent of methanol, 13 per cent 35 of isobutyl alcohol, 15 per cent of higher alcohols, ketones and the like.

The above examples are only given for the 40 purpose of illustration and the invention is not limited thereto.

What I claim is:

1. A composition of matter substantially composed of gasoline and not more than 12 45 per cent by volume of the gasoline of crude synthetic methanol containing products of a higher order than methanol.

2. A composition of matter comprising gasoline and between about 4 and 12 per cent 50 by volume of the gasoline of crude synthetic

WILHELM GAUS. 55

60

65

70

75

80

85

90

95

100